

## UNITED STATES PATENT OFFICE

2,373,733

## STEAM CYLINDER LUBRICANTS

Elmer Wade Adams, Hammond, and Frederick H. MacLaren, Munster, Ind., assignors to Standard Oil Company, Chicago, Ill., a corporation of Indiana

No Drawing. Application May 27, 1944,  
Serial No. 537,736

9 Claims. (Cl. 252—53)

This invention relates to lubricants for valves or other mechanical parts exposed to steam and more particularly to steam cylinder lubricants and the like.

The principal problem of lubrication of steam engines is that of lubricating the internal parts where the greatest frictional losses and wear occur. The problem which is peculiar to the steam engine lubrication and introduces factors seldom encountered elsewhere is due to the fact that lubrication must be accomplished on frictional surfaces in direct contact with or swept by steam. In direct contact with the steam are the working surfaces of the cylinder, the piston and piston ring, the valves for admitting and exhausting steam, and the connecting rod and valve rods. Steam varying in the properties it acquires when produced and in the properties it assumes during use sweeps in and out of the cylinder on each stroke of the piston and adds to the difficulty of securing good lubrication. These factors require that the steam cylinder be preferentially wetted with oil rather than with the water resulting from steam condensation and for this reason lubricants employed in steam cylinders must be capable of rapidly forming an invert emulsion with the steam. While the steam cylinder lubricant must be one which readily atomizes and mixes with the steam and leaves a tenacious film which resists subsequent displacement by water, the oil carried over with the steam must be one which separates satisfactorily from the exhaust steam. The oil must also be one which is resistant to oxidation and to the formation of objectional deposits.

In our copending application Serial No. 432,834, filed February 28, 1942, of which the present application is a continuation-in-part, we disclose a steam cylinder lubricant comprising a blend of a relatively viscous mineral oil, preferably a heavy steam refined lubricating oil and small amounts of a fatty material such as lard oil and a complex glyceride phosphoric acid ester, for example lecithin. The phosphatidic material in the steam cylinder lubricant disclosed in our copending application is a highly desirable constituent since it is a very effective invert emulsifier. It has been discovered, however, that under certain conditions steam cylinder oils in which the phosphatidic material is the sole agent for producing

an invert emulsion performed unsatisfactorily due to the high detergency effect of the lecithin. This results in dry pistons and cylinder walls and reduces the effectiveness of the compounded oil as a lubricant. Furthermore, it has been found that under certain conditions this lubricant did not separate satisfactorily from the exhaust steam.

It is therefore an object of the present invention to provide a steam cylinder lubricant which will readily form a stable invert emulsion and which at the same time does not possess too great detergency properties.

Another object of the present invention is to provide a steam cylinder lubricant which will readily form a stable invert emulsion and which will maintain a continuous resistant lubricating oil film on or between the metal surfaces to be lubricated.

Another object of the present invention is to provide a steam cylinder lubricant which will quickly atomize and mix with steam.

Still another object of the invention is to provide a steam cylinder lubricant which will separate satisfactorily from exhaust steam.

A still further object of the invention is to provide a steam cylinder oil which is resistant to oxidation and to the formation of objectionable deposits.

Other objects and advantages of the invention will become apparent from the following description thereof.

We have discovered that a steam cylinder oil capable of rapidly forming invert emulsions when mixed with steam, which is stable and which maintains a continuous resistant lubricating film is obtained by compounding a relatively viscous mineral oil with small amounts of a fatty material, preferably a fatty oil, a complex glyceride phosphoric acid ester and a residuum having a Furol viscosity at 210° F. of from about 750 seconds to about 950 seconds obtained from a naphthenic crude petroleum oil or from a crude petroleum which is predominantly naphthenic.

The mineral oil constituent is preferably a viscous oil having a Saybolt Universal viscosity at 210° F. of from about 100 seconds to about 300 seconds and preferably from about 150 seconds to about 250 seconds. For example, the oil may be a heavy steam refined Mid-continent lubricat-

ing oil having a flash point of about 530° F. and a Saybolt Universal viscosity at 210° F. of about 200 seconds or it can be a heavy Pennsylvania steam refined oil having a Saybolt Universal viscosity at 210° F. of about 220 seconds. While the oil is preferably a steam refined residual oil, blends of residual oils and distillates to give the desired viscosity can also be employed.

The fatty material or fatty oil such as tallow, lard oil, animal fat, beta fat and the like can be employed in quantities ranging from about 5% to about 10% and preferably from about 7% to about 9%.

The complex glyceride phosphoric acid ester can be a phosphatide such as lecithin, cephalin and the like. While substantially chemically pure phosphatidic materials can be employed, commercial grades of phosphatides or commercial lecithin products known by the trade names of "Lipoidol," "Soyab," "Colloidal HX" and others are suitable. The phosphatidic material can be employed in amounts of from about 0.05% to about 1% and preferably from about .1% to about .5%.

The other constituent of the herein described steam cylinder lubricant which functions to form invert emulsions is a residuum petroleum oil having a furol viscosity at 210° F. of from about 750 seconds to about 950 seconds and preferably from about 850 seconds to about 900 seconds obtained from naphthenic petroleum oils or from petroleum oils which are predominantly naphthenic. Residuums suitable for this purpose are those obtained from Smackover crude oil or crude oil having properties similar thereto. The residuum oil can be employed in quantities within the range of from about 1% to about 5% and preferably from about 2% to about 4%.

The following formulas are specific examples of compounded steam cylinder lubricants made in accordance with the present invention.

|                        | I        | II       | III      |
|------------------------|----------|----------|----------|
|                        | Per cent | Per cent | Per cent |
| Petroleum oil          | 187.3    | 289.4    | 198.4    |
| Fatty oil (lard oil)   | 8.5      | 8.5      | 8.5      |
| Petroleum residuum     | 4.0      | 2.0      | 2.0      |
| Phosphatide (lecithin) | 0.2      | 0.1      | 0.1      |

<sup>1</sup> M. C. oil—S. U. V. at 210° F.—165 seconds.

<sup>2</sup> M. C. steam refined oil—S. U. V. at 210° F.—200 seconds.

<sup>3</sup> Pennsylvania steam refined oil—S. U. V. at 210° F.—220 seconds.

<sup>4</sup> Residuum from Smackover crude oil—furol viscosity at 210° F.—800-900 seconds.

By the proper balancing of the phosphatidic material and the residuum oil to maintain both adequate invert emulsifying properties and the desired detergent characteristics, a greatly improved steam cylinder lubricant is obtained.

In evaluating steam cylinder oils, the rapidity with which the oil is capable of forming a substantially rigid emulsion is determined. One method by which this factor is determined is by the so-called MacLaren steam cylinder emulsion test. In this test 20 ccs. of tap water and 30 ccs. of the oil to be tested are placed in a glass stoppered 50 cc. graduate and the contents thereof, with the stopper removed, is heated for 45 minutes in a water bath maintained at a temperature of about 165° F. to 175° F. The graduate is then removed from the water bath, stoppered and inverted three or four times, releasing the pressure each time. The graduate is then shaken vigorously and the time noted and recorded in seconds for a rigid emulsion to form. Oil compositions which fail to form a rigid emulsion with

3 minutes of vigorous shaking are unsuitable as steam cylinder lubricants.

The effect of naphthenic petroleum residuums in reducing the time for a rigid emulsion to form in the above test is demonstrated by the following data:

|                                                                      | Oil composition | Time (seconds) for rigid emulsion to form |
|----------------------------------------------------------------------|-----------------|-------------------------------------------|
| 91.5% Pa. steam refined oil (S. U. V. at 210° F.—220 seconds)        | 300             |                                           |
| 8.5% lard oil                                                        | 150             |                                           |
| 91.0% Pa. steam refined oil (S. U. V. at 210° F.—220 seconds)        | 150             |                                           |
| 8.5% lard oil                                                        | 45              |                                           |
| 0.5% lecithin                                                        | 45              |                                           |
| 89.4% Pa. steam refined oil (S. U. V. at 210° F.—220 seconds)        | 360+            |                                           |
| 8.5% lard oil                                                        | 240             |                                           |
| 0.1% lecithin                                                        | 95              |                                           |
| 2.0% Smackover residuum (furol viscosity at 210° F.—800-900 seconds) | 75              |                                           |
| 91.5% M. C. steam refined oil (S. U. V. at 210° F.—210 seconds)      | 240             |                                           |
| 8.5% lard oil                                                        | 240             |                                           |
| 0.5% lecithin                                                        | 240             |                                           |
| 89.4% M. C. steam refined oil (S. U. V. at 210° F.—200 seconds)      | 95              |                                           |
| 8.5% lard oil                                                        | 95              |                                           |
| 0.1% lecithin                                                        | 95              |                                           |
| 2.0% Smackover residuum (furol viscosity at 210° F.—800-900 seconds) | 95              |                                           |
| 87.3% M. C. steam refined oil (S. U. V. at 210° F.—165 seconds)      | 75              |                                           |
| 8.5% lard oil                                                        | 75              |                                           |
| 0.2% lecithin                                                        | 75              |                                           |
| 4.0% Smackover residuum (furol viscosity at 210° F.—800-900 seconds) | 75              |                                           |

35 The above data show that the addition of the naphthenic petroleum residuum materially reduces the time to form rigid emulsions by the MacLaren test.

40 The effectiveness of steam cylinder lubricants made in accordance with the present invention is further demonstrated by the results obtained in numerous commercial installations.

45 Steam cylinder lubricants compounded in accordance with the present invention have been subjected to field service tests in engines over long periods of time and in most cases under extremely adverse steam conditions. Closely observed tests were conducted on twenty-six engines

50 including uniflow as well as Corliss, slide and piston valve types. These engines ranged in size from 7" x 12" running at 300 R. P. M. to 20" x 40" x 42" cross-compound running at about 103 R. P. M. with steam pressure ranging from 100 pounds

55 saturated steam to 230 pounds with 100° superheat. The results of these tests demonstrate that the herein described steam cylinder oils atomized more readily than conventional steam cylinder oils and permitted the use of higher viscosity oils

60 resulting in lower oil feed rates. These tests further demonstrated that our improved steam cylinder oils separated satisfactorily from the exhaust steam and in sixteen cases of the twenty-six test installations, the oil separated from the

65 exhaust steam so well that the latter was used for processing in laundries, paper mills, building heat, dried milk plants, and cheese factories. The tests further demonstrated that the steam cylinder oils of the present invention were stable against the formation of objectionable deposits resulting in freedom from plugged quills, and therefore permitted longer operations without the necessity of shut-downs.

70 Since the steam cylinder oils of the present invention readily atomize with steam, it is possible

to use more viscous oils which accordingly permit lower oil feed rates. By a proper balance of the phosphatidic material and the naphthenic residuum, we have obtained a steam cylinder lubricant which, while readily emulsifying with steam, nevertheless separates from the exhaust steam without difficulty so that the exhaust steam can be employed for other purposes such as for processing. This is not possible when the steam cylinder oil employed does not separate satisfactorily from the exhaust steam.

While we have described our invention by references to specific preferred embodiments thereof, the same have been given by way of illustration and not intended to limit the scope of our invention except in so far as the same is defined by the following claims.

We claim:

1. A steam cylinder oil comprising a hydrocarbon lubricating oil having a Saybolt Universal viscosity at 210° F. within the range of about 100 seconds to about 300 seconds, from about 5% to about 10% of a fatty oil, from about 1% to about 5% of a petroleum residuum having a furol viscosity at 210° F. of from about 750 seconds to about 950 seconds, obtained from a naphthenic type crude petroleum oil, and from about 0.05% to about 1% of a complex glyceride phosphoric acid ester.

2. A steam cylinder oil as described in claim 1 in which the fatty oil is lard oil and the complex glyceride phosphoric ester is a phosphatide.

3. A steam cylinder oil as described in claim 1 in which the complex glyceride phosphoric acid ester is lecithin.

4. A steam cylinder oil which forms water-in-oil emulsions comprising a hydrocarbon lubricating oil having a Saybolt Universal viscosity at 210° F. of from about 100 seconds to about 300 seconds, from about 7% to about 9% of a fatty oil, from about 0.1% to about 0.5% of a complex glyceride phosphoric acid ester, and from about 2% to about 4% of a residuum petroleum oil having a furol viscosity at 210° F. of from about 800 seconds to about 900 seconds obtained from a predominantly naphthenic petroleum oil.

5. A steam cylinder oil as described in claim 4 in which the fatty oil is lard oil, the complex glyceride phosphoric acid ester is lecithin, and the residuum is a residuum obtained from a Smackover type crude oil.

6. A steam cylinder oil comprising a Pennsylvania steam refined mineral oil having a Saybolt Universal viscosity at 210° F. of about 220 seconds, 8½% lard oil, 0.1% of a phosphatidic material, and 2% of a residuum petroleum oil having a furol viscosity at 210° F. of about 800 to 900 seconds obtained from a crude petroleum oil of the Smackover type.

7. A steam cylinder oil comprising a steam refined Mid-continent mineral oil having a Saybolt Universal viscosity at 210° F. of from about 165 seconds to about 200 seconds, about 8½% of lard oil, from about 0.1% to about 0.2% lecithin, and from about 2% to about 4% of a residuum petroleum oil having a furol viscosity at 210° F. of about 800-900 seconds obtained from a crude petroleum oil of the Smackover type.

8. In the lubrication of cylinders of steam engines the improvement comprising commingling with the steam supplied to such cylinders a lubricant comprising a hydrocarbon oil having a Saybolt Universal viscosity at 210° F. of from about 100 seconds to about 300 seconds, from about 5% to about 10% of a fatty oil, from about 0.05% to about 1% of a complex glyceride phosphoric acid ester, and from about 1% to about 5% of a residuum petroleum oil having a furol viscosity at 210° F. of from about 750 seconds to about 950 seconds obtained from a predominantly naphthenic petroleum oil, whereby an invert emulsion which preferentially wets the surfaces of the cylinders is formed with the steam.

9. The lubrication of cylinders of steam engines as described in claim 8 in which the fatty oil is lard oil, the complex glyceride phosphoric acid ester is a phosphatide, and the petroleum residuum is a residuum obtained from a crude oil of the Smackover type.

ELMER WADE ADAMS.  
FREDERICK H. MACLAREN.

CERTIFICATE OF CORRECTION.

Patent No. 2,373,733.

April 17, 1945.

ELMER WADE ADAMS, ET AL.

It is hereby certified that error appears in the printed specification of the above numbered patent requiring correction as follows: Page 2, first column, line 47, in the table, fourth column thereof, for "98.4" read --89.4--; and that the said Letters Patent should be read with this correction therein that the same may conform to the record of the case in the Patent Office.

Signed and sealed this 19th day of June, A. D. 1945.

Leslie Frazer

(Seal)

Acting Commissioner of Patents.